

July 18, 1933.

L. W. LARSON

1,918,849

MOTHPROOF MOHAIR

Filed March 20, 1931

Fig. 1.



Fig. 2.



Fig. 3.



Inventor  
Lourie W. Larson

By Chindahl, Parker & Baldwin  
Atty's.

## UNITED STATES PATENT OFFICE

LOURIE W. LARSON, OF CHICAGO, ILLINOIS

## MOTH-PROOF MOHAIR

Application filed March 20, 1931. Serial No. 524,199.

This invention relates to that class of upholstering material such as mohair subject to attack by moths, and the general object is to render such a fabric moth-proof by forming on the back or underside thereof a coating of vegetable material such as cotton fibers which effectually protect the animal fibers of the mohair from the attack of moths or the larvae thereof.

10 Another object is to provide a coating of the above character which is simple and inexpensive to apply, which does not reduce the flexibility of the fabric, and which is unbroken by the stretching of the fabric incident to its use in upholstering.

Other objects and advantages of the invention will become apparent from the following detailed description taken in conjunction with the accompanying drawing in which:

20 Figure 1 shows on an enlarged scale a piece of fabric such as mohair viewed from the underside and having a portion thereof treated in accordance with the present invention.

25 Fig. 2 is a sectional view of the mohair shown in Fig. 1 but on a greatly enlarged scale.

Fig. 3 is an enlarged view of one of the bundles of hair bent into the shape which 30 it resumes in the weaving process.

While the invention is susceptible of various modifications and alternative constructions, I have shown in the drawing and will herein describe in detail the preferred embodiment, but it is to be understood that I do not thereby intend to limit the invention to the specific form disclosed, but intend to cover all modifications and alternative constructions falling within the spirit and scope 40 of the invention as expressed in the appended claims.

As shown in the drawing, modern mohair consists of a facing comprising bundles 5 (Fig. 3) of relatively short animal fibers such as goat's-hair bent into substantially U-shape with their intermediate portion passing beneath a warp thread 6, then over two warp threads 7, and finally under a third warp thread 8, all of which warp threads are held together by cross threads 9. Thus the

free ends of the bundle of fibers are held in parallel relation by a cloth backing formed by the warp threads and the threads 9. When the cloth is thus woven, the bights 10 of the fiber bundles are exposed on the back side of the mohair. Moths and their larvae attack the fabric by boring through from the front and then turning to work on the back side of the fiber when the latter is used in upholstering. Their attack is centered upon the bights 10 which when completely severed by the moths allow the ends of the bundles to be pulled out of the warp threads leaving the latter bare.

Referring now to Figs. 1 and 2, the invention in its preferred form contemplates the covering of the back surface of the mohair cloth formed as above described with a thin coextensive coating or backing 12 of cotton fibers which are so closely matted together that the bights 10 of the hair bundles are effectually covered.

In manufacture, the coating 12 may be formed by first covering the back surface of the mohair cloth with a suitable adhesive 11. Then the cotton fibers are pressed against the adhesive which retains a sufficient quantity of the fiber to form the coating 12 which, being composed of vegetable material, entangle the nippers of the moths and cannot be penetrated by them. The mohair is thus rendered moth-proof.

Inasmuch as the protecting fibers of the coating 12 are merely matted together, the flexibility of the mohair is not impaired materially. Such a coating permits the mohair to be stretched readily as is necessarily done in upholstering and remains intact after such stretching. The thickness of the mohair is not materially increased with such a moth-proof coating and can be folded as may be required without leaving bulky seams.

Instead of using an adhesive as above described, the cotton fibers constituting the protecting coating may be woven directly into the mohair and so held by the warp threads and the threads 9 that they will cover the bights 10 of the hair bundles which would otherwise be exposed on the underside of the mohair.

It has been found that mohair treated in the manner above described will not be attacked by moths when used in upholstery. The treatment is simple and inexpensive and does not interfere in any way with the ordinary use of the mohair.

I claim as my invention:

1. A moth-proof fabric of the character set forth having an animal fiber facing, and a

thin flexible unwoven backing coextensive with the facing and composed of matted cotton fibers.

2. A moth-proof mohair fabric having an unwoven backing composed of a thin flexible sheet of cotton fibers matted together and coextensive with the fabric.

LOURIE W. LARSON.

75

10

15

80

20

85

25

90

30

95

35

100

40

105

45

110

50

115

55

120

60

125

65

130

**CERTIFICATE OF CORRECTION.**

**Patent No. 1,918,849.**

**July 18, 1933.**

**LOURIE W. LARSON.**

**It is hereby certified that error appears in the above numbered patent requiring correction as follows: In the grant, drawing, and in the heading to the specification, title of invention, for the words "Moth-Proof Mohair" read "Moth-Proof Fabric"; and that the said Letters Patent should be read with this correction therein that the same may conform to the record of the case in the Patent Office.**

**Signed and sealed this 29th day of August, A. D. 1933.**

**M. J. Moore.**

**(Seal)**

**Acting Commissioner of Patents.**